# EUROPEAN PATENT SPECIFICATION

(11) **EP 0 407 977 B1**
(45) Date of publication and mention of the grant of the patent: **28.04.1993**
(21) Application number: 90113167.2
(22) Date of filing: 10.07.1990
(51) Int. Cl.: C10M 141/10

(54) **Lubricating oil composition**
Schmierölzusammensetzung
Composition d'huile lubrifiante

(30) Priority: 13.07.1989 JP 178937/89
(43) Date of publication of application: 16.01.1991
(73) Proprietor: IDEMITSU KOSAN COMPANY LIMITED, Tokyo 100 (JP)
(72) Inventor: Hata, Hitoshi, c/o Idemitsu Kosan Co. Ltd., Ichihara-shi, Chiba-ken (JP)
(74) Representative: Strehl Schübel-Hopf Groening & Partner

(56) References cited:
- EP-A- 0 113 045
- EP-A- 0 280 260
- EP-A- 0 286 996
- EP-A- 0 291 006
- DE-A- 1 956 638
- US-A- 2 418 894
- US-A- 2 945 810

## Description

### (a) Field of the Invention

The present invention relates to a lubricating oil composition which can be suitably used as hydraulic fluid, traction fluid, bearing oil, gear oil, engine oil, etc.

### (b) Description of the Related Art

Zinc dithiophosphates have been widely used in lubricating oils having requirements for the function of improving wear resistance and load carrying capacity, thermostability, and oxidation stability.

Recently, as the service environment of these lubricating oils has become severe, there has arisen a demand particularly for lubricating oils having such high thermostability and oxidation stability as to withstand use at high temperature.

As a means of improving thermostability and oxidation stability, it is proposed in Japanese Patent Application Kokai Koho (Laid-open) No. 60-248796 to add zinc dithiophosphates into lubricating base oils together with other additives including nitrogen-containing copolymers, metallic detergent-dispersants, ashless detergent-dispersants, etc. However, such additives decrease load carrying capacity and wear resistance and cannot bring about sufficient increase in thermostability and oxidation stability, and therefore, the obtained lubricating oil cannot be prevented sufficiently from formation of sludge and coloration and discoloration.

EP-A-0 280 260 discloses a lubricating oil composition comprising (A) a mineral oil having a specific viscosity and viscosity index, (B) 0.5 to 20 % by weight of an ethylene-a-olefin copolymer having a specific number average molecular weight, (C) 0.05 to 20 % by weight of polymethacrylate having a specific number average molecular weight or a mixture of said polymethacrylate and an olefin copolymer, and either (D-I) 1 to 20 % by weight of a detergent-dispersant and/or an antioxidant, or (D-II) 0.5 to 20 % by weight of at least one member selected from the group consisting of an extreme pressure agent, an anti-wear agent and an oiliness agent. As one suitable antioxidant, among others, zinc dithiophosphate, and as one suitable oiliness agent, among others, oleyl alcohol are disclosed. Zinc dithiophosphate is also mentioned, besides others, as extreme pressure agent. The above lubricating oil composition is useful as a multi grade lubricating oil composition which is excellent in shear stability.

EP-A-0 291 006 discloses a lubricating oil composition containing (A) a base oil having a specific viscosity, pour point and viscosity index, (B) an ethylene-α-olefin copolymer having a specific number average molecular weight, and (C) at least one additive selected from an extreme pressure agent, an anti-wear agent, an oiliness agent and a detergent dispersant. Among other useful compounds, oleyl alcohol is mentioned as being suited as oiliness agent. Furthermore, zinc dithiophosphate is mentioned besides numerous other compounds as compound suited as extreme pressure agent, or as a further additive for preventing oxidation.

This oil composition exhibits a high viscosity index and good temperature characteristics, particularly at low temperatures and is further excellent in shear stability and other properties, such as wear resistance and detergency.

The present invention has been made under the above-described circumstances, and the object of the present invention is to provide a lubricating oil composition which has not only excellent effect in improving load carrying capacity and wear resistance but also excellent thermostability and oxidation stability whereby formation of sludge and coloration and discoloration are inhibited and heat degradation and oxidation degradation can be retarded.

We have made study diligently for solving the above-described problems and have found that a lubricating oil composition satisfying the above-described object is obtainable by blending unsaturated aliphatic alcohols of from 16 to 24 carbon atoms together with zinc dithiophosphates into lubricating base oils in a specific ratio, and on the basis of the finding, we have eventually completed the present invention.

That is, the present invention provides a lubricating oil composition, comprising:
(A) a major amount of at least one lubricating base oil;
(B) from 0.05 to 5 % by weight of at least one zinc dithiophosphate having a structure represented by the following general formula (1) wherein each of R¹, R², R³, and R⁴ is independently a primary alkyl group of from 2 to 30 carbon atoms, a secondary alkyl group of from 3 to 30 carbon atoms, a cycloalkyl group of from 6 to 30 carbon atoms, an aryl group of from 6 to 14 carbon atoms or an alkylaryl group of from 7 to 30 carbon atoms;
   and
(C) from 0.01 to 10 % by weight of at least one unsaturated aliphatic alcohol of from 16 to 24 carbon atoms,
   wherein the weight ratio of the unsaturated aliphatic alcohol to the zinc dithiophosphate, (C)/(B), is from 0.1 to 10.

The oxidation stability of the lubricating oil composition of the present invention can be further improved by adding detergent-dispersants. That is, the present invention also provides a lubricating oil composition, comprising:
(A) a major amount of at least one lubricating base oil;
(B) from 0.05 to 5 % by weight of at least one zinc dithiophosphate having a structure represented by the following general formula (1) wherein R¹, R², R³, and R⁴ are as defined above;
(C) from 0.01 to 10 % by weight of at least one unsaturated aliphatic alcohol of from 16 to 24 carbon atoms; and
(D) from 0.01 to 5.0 % by weight of at least one detergent-dispersant,
wherein the weight ratio of the unsaturated aliphatic alcohol to the zinc dithiophosphate, (C)/(B), is from 0.1 to 10.

The lubricating oil composition of the present invention can be suitably used as hydraulic fluid, traction fluid, bearing oil, gear oil, engine oil, etc. even in severe circumstances where exposure to high temperature is inevitable.

The component (A), i.e. the lubricating base oil to be used in the lubricating oil composition of the present invention may be any one generally used in lubricating oils and is not particularly limited. Generally, a mineral oil or a synthetic detail each having a kinematic viscosity of from 5 to 10,000$\frac{\text{mm²}}{\text{s}}$ (cSt) as measured at 40 °C may be used

The mineral oil is not particularly limited so far as it satisfies the above-described condition, and some examples include those obtained by refining lubricating oil fraction of petroleum by means of solvent refining, hydrorefining, clay treatment, or a combination thereof and highly aromatic fractions obtained by solvent refining of lubricating oils, or hydrogenation products of the highly aromatic fractions. Some examples of the synthetic oil include alkyl-substituted aromatic compounds, poly-α-olefin oils, ester oils, diester oils, hindered ester oils, synthetic naphthene oils, polyglycol oils, and mixtures thereof.

The zinc dithiophosphate (ZnDTP) to be used as the component (B) in the lubricating oil composition of the present invention is the compound represented by the following general formula (I)
wherein each of R¹, R², R³, and R⁴ is independently a primary alkyl group of from 2 to 30 carbon atoms, preferably from 3 to 12 carbon atoms, a secondary alkyl group of from 3 to 30 carbon atoms, preferably from 3 to 12 carbon atoms, a cycloalkyl group of from 6 to 30 carbon atoms, an aryl group of from 6 to 14 carbon atoms or an alkylaryl group of from 7 to 30 carbon atoms, preferably from 9 to 24 carbon atoms.

Some examples of the zinc dithiophosphate include
zinc dialkyldithiophosphates, such as
zinc di-n-propyldithiophosphate,
zinc diisopropyldithiophosphate,
zinc di-n-butyldithiophosphate,
zinc diisobutyldithiophosphate,
zinc di-sec-butyldithiophosphate,
zinc di-n-amyldithiophosphate,
zinc diisoamyldithiophosphate,
zinc di-n-hexyldithiophosphate,
zinc di-sec-hexyldithiophosphate,
zinc bis(2-ethylhexyl)dithiophosphate, and
zinc didecyldithiophosphate,
zinc diaryldithiophosphates, such as
zinc diphenyldithiophosphate, and
zinc bis(alkylaryl)dithiophosphates, such as
zinc bis(octylphenyl)dithiophosphates,
zinc bis(nonylphenyl)dithiophosphates, and
zinc bis(dodecylphenyl)dithiophosphates.

The above-described component (B) i.e. the zinc dithiophosphate is present in the lubricating oil composition of the present invention at a concentration of from 0.05 to 5.0 % by weight, preferably from 0.1 to 3.0 % by weight. If the percentage of the component (B) is less than 0.05 % by weight of the lubricating oil composition, the effect of improving wear resistance and load carrying capacity will be small. On the other hand, even if the percentage of the component (B) exceeds 5.0 % by weight of the lubricating oil composition, larger effect cannot be expected.

The unsaturated aliphatic alcohol of from 16 to 24 carbon atoms which is to be used as the component (C) in the lubricating oil composition of the present invention may be any alcohol having the above-described number of carbon atoms and at least one double bond in each molecule. The preferred are alcohols having an iodine number of about not less than 50. Some examples of the preferred unsaturated aliphatic alcohols include cis-11-hexadecene-1-ol (C₁₆H₃₂O), cis-9-octadecene-1-ol (oleyl alcohol, C₁₈H₃₆O), 3,7,11,15-tetramethyl-2-hexadecene-1-ol (C₂₀H₄₀O), 9-eicosene-1-ol (C₂₀H₄₀O), 11-docosene-1-ol (C₂₂H₄₄O), 13-docosene-1-ol (C₂₂H₄₄O), 12-tetracosene-1-ol (C₂₄H₄₈O), and 13-tetracosene-1-ol (C₂₄H₄₈O).

Among these, the particularly preferred examples include 11-docosene-1-ol, 13-docosene-1-ol, 9-eicosene-1-ol, and cis-9-octadecene-1-ol (oleyl alcohol).

The above-described component (C), i.e. the unsaturated aliphatic alcohol is present in the lubricating oil composition of the present invention at a concentration of from 0.01 to 10 % by weight, preferably from 0.05 to 6.0 % by weight, and the weight ratio of the unsaturated aliphatic alcohol to the zinc dithiophosphate, (C)/(B) is from 0.1 to 10, preferably from 0.2 to 3.0. If the percentage of the component (C) in the lubricating oil composition is less than 0.01 % by weight or (C)/(B) is less than 0.1, the component (C) cannot produce much effect of inhibiting the formation of sludge. On the other hand, even if the percentage of the component (C) exceeds 10 % by weight or (C)/(B) exceeds 3.0, larger effect cannot be expected.

The oxidation stability of the lubricating oil composition of the present invention comprising the above-described lubricating base oil (A), the component (B), and the component (C), can be further improved by adding a relatively small amount of at least one detergent-dispersant (component D).

The detergent-dispersant to be used in the present invention may be any known detergent-dispersant, and some examples include metallic detergent-dispersants such as petroleum sulfonates, phosphonates, and phenates, and ashless detergent-dispersants, such as succinic acid derivatives and amine-type detergent-dispersants. Some typical examples of the detergent-dispersants which may be suitably used are Ca sulfonate and Ca phenate. The component (D), i.e. the detergent-dispersant is present in the lubricating oil composition of the present invention at a concentration of from 0.01 to 5.0 % by weight, preferably from 0.1 to 1.5 % by weight, more preferably from 0.2 to 1.0 % by weight.

The above-described lubricating oil composition of the present invention comprising the lubricating base oil (A), component (B), and component (C) or the lubricating base oil (A), component (B) component (C) and component (D) may further contain a relatively small amount of at least one additive compound (component E) selected from the group consisting of phosphoric esters, phosphorous esters, amine salts of phosphoric esters, and amine salts of phosphorous esters.

Some examples of the phosphoric esters and the phosphorous esters which may be suitably used are the compounds represented by the following general formulas (II) and (III) respectively:
wherein each of R⁵, R⁶, R⁷, R⁸, R⁹, and R¹⁰ is, for example, independently a hydrogen atom, an alkyl group of from 4 to 30 carbon atoms, an aryl group of from 6 to 30 carbon atoms, or an alkylaryl group of from 7 to 30 carbon atoms, and two or more of them may be identical with each other or they may be different from each other.

Some typical examples of the phosphoric esters and the phosphorous esters include triphenyl phosphate, tricresyl phosphate, trixylenyl phosphate, tris(isopropylphenyl)phosphate, butyl acid phosphate, 2-ethylhexyl acid phosphate, lauryl acid phosphate, oleyl acid phosphate, stearyl acid phosphate, dibutyl hydrogen phosphite, dioctyl hydrogen phosphite, dioleyl hydrogen phosphite, and distearyl hydrogen phosphite.

Some examples of the amine salts of phosphoric esters and the amine esters of phosphorous esters include lauryl amine salt, oleyl amine salt, coconut amine salt, and beef tallow amine salt

The component (E), i.e. the additive compound is present in the lubricating oil composition of the present invention at a concentration of from 0.01 to 5.0 % by weight, preferably from 0.1 to 1.5 % by weight, more preferably from 0.2 to 1.0 % by weight. Addition of the component (E) improves wear resistance still more.

Further, the lubricating oil composition of the present invention may contain other additives which has been generally added into lubricating oils, for example, antioxidants, viscosity index improvers, corrosion inhibitors, rust-preventive agents, metal deactivators, or antifoaming agents.

The following Examples are given to illustrate the present invention in more detail. The scope of the invention is not, however, meant to be limited to the specific details of these Examples.

### EXAMPLES 1 TO 14 AND COMPARATIVE EXAMPLES 1 TO 5

Table 1 shows the composition and the test results of the lubricating oil compositions of the Examples and Comparative Examples.

The tests made in the Examples and Comparative Examples were carried out by means of the following methods.

### (1) Coloration and Discoloration, (2) Property of Inhibiting Formation of Sludge

These properties were examined according to JIS K 2540, Method of Testing the Thermostability of Lubricating Oils, at a testing temperature (oil temperature) of 140 °C. The catalysts used were copper wire, iron wire, and aluminum wire each being ⌀ 1.6 mm × 8 cm.

Evaluation of the coloration and discoloration (1) was carried out by removing the sample used every 24 hour to observe the color of the sample (ASTM JIS K 2580) and is shown as the time (h) required of the color to exceed the ASTM color grade 4. Evaluation of the property of inhibiting formation of sludge was carried out by observing the above-described sample and was shown as the time (h) required of the deposition of separated material to be observed.

### (3) Oxidation Stability

Oxidation stability was examined according to JIS K 2514, paragraph 3.1, Method of Testing the Oxidation Stability of Lubricating Oils for Internal Combustion Engines (so called ISOT).

### Conditions of ISOT

The condition for the samples from Example 2 and Comparative Example 1 were @165.5 °C × 24 h, and the condition for the sample from Example 12 was @150 °C × 96 h.

### (4) Wear Resistance (Falex wear resistance)

The examination of wear resistance was conducted according to ASTM-D 2670.

The marks shown in Table 1 have the following meaning

Table 1 shows that the addition of the component (C) such as 13-docosene-1-ol and oleyl alcohol, i.e., in particular, unsaturated aliphatic alcohols of from 18 to 22 carbon atoms improved thermostability and oxidation stability, and particularly, the properties of inhibiting coloration, discoloration, and formation of sludge were remarkably improved. As apparent from Comparative Examples 4 and 5, the compounds other than the components of the present invention could not produce the directed effects.

## Claims

1. A lubricating oil composition, comprising:
(A) a major amount of at least one lubricating base oil;
(B) from 0.05 to 5 % by weight of at least one zinc dithiophosphate having a structure represented by the following general formula (1) wherein each of R¹, R², R³, and R⁴ is independently a primary alkyl group of from 2 to 30 carbon atoms, a secondary alkyl group of from 3 to 30 carbon atoms, a cycloalkyl group of from 6 to 30 carbon atoms, an aryl group of from 6 to 14 carbon atoms or an alkylaryl group of from 7 to 30 carbon atoms;
and
(C) from 0.01 to 10 % by weight of at least one unsaturated aliphatic alcohol of from 16 to 24 carbon atoms,
wherein the weight ratio of the unsaturated aliphatic alcohol to the zinc dithiophosphate, (C)/(B), is from 0.1 to 10.

2. A lubricating oil composition according to claim 1 which additionally comprises:
(D) from 0.01 to 5.0% by weight of at least one detergent-dispersant.

3. The lubricating oil composition as claimed in claim 1 or 2, wherein the lubricating base oil is a mineral oil having a kinematic viscosity of from 5 to 10,000$\frac{\text{mm²}}{\text{s}}$ (cSt) as measured at 40°C or a synthetic oil having a kinematic viscosity of from 5 to 10,000$\frac{\text{mm²}}{\text{s}}$ (cSt) as measured at 40°C.

4. The lubricating oil composition as claimed in any of the claims 1 to 3, wherein the zinc dithiophosphate is selected from the group consisting of zinc di-primary-(C₃-C₁₂)-alkyldithiophosphates, zinc-di-secondary-(C₃-C₁₂)-alkyldithiophosphates, and zinc-bis-(C₉-C₂₄)-(alkylaryl)dithiophosphates.

5. The lubricating oil composition as claimed in any of the claims 1 to 4, wherein the unsaturated aliphatic alcohol is 11-docosene -1-ol, 13-docosene-1-ol, 9-eicosene-1-ol or cis-9-octadecene -1-ol.

6. The lubricating oil composition as claimed in claim 1 or 5, wherein the unsaturated aliphatic alcohol is 13-docosene -1-ol or cis-9-octadecene-1-ol.

7. The lubricating oil composition as claimed in claim 1, wherein the lubricating base oil is a mineral oil, the zinc dithiophosphate is a mixture of zinc di-primary-(C₄-C₆)-alkyldithiophosphates, and the unsaturated aliphatic alcohol is cis-9-octadecene-1-ol.

8. The lubricating oil composition as claimed in any of the claims 1 to 7, further comprising (E) from 0.01 to 5.0% by weight of at least one additive compound selected from the group consisting of phosphoric esters, phosphorous esters, amine salts of phosphoric esters, and amine salts of phosphorous esters.

9. The lubricating oil composition as claimed in claim 2, wherein the unsaturated aliphatic alcohol is 13-docosene -1-ol.

10. The lubricating oil composition as claimed in claim 2, wherein the lubricating base oil is a mineral oil, the zinc dithiophosphate is a mixture of zinc di-primary-(C₄-C₆)-alkyldithiophosphates, the unsaturated aliphatic alcohol is 13-docosene-1-ol, and the detergent-dispersant is a mixture of Ca sulfonate and Ca phenate.

11. The lubricating oil composition as claimed in claim 2, wherein the lubricating base oil is a mineral oil, the zinc dithiophosphate is a mixture of zinc di-primary -(C₄-C₆)-alkyldithiophosphates, the unsaturated aliphatic alcohol is 13-docosene-1-ol, the detergent-dispersant is a mixture of Ca sulfonate and Ca phenate, and the additive compound is tricresyl phosphate.

## Patentansprüche

1. Schmierölzusammensetzung, enthaltend
(A) einen Hauptanteil mindestens eines Grundschmieröls,
(B) 0,05 bis 5 Gew.-% mindestens eines Zinkdithiophosphats einer Struktur, die durch die folgende allgemeine Formel (1) dargestellt ist in der jeder der Reste R¹, R², R³ und R⁴ unabhängig eine primäre Alkylgruppe mit 2 bis 30 Kohlenstoffatomen, eine sekundäre Alkylgruppe mit 3 bis 30 Kohlenstoffatomen, eine Cycloalkylgruppe mit 6 bis 30 Kohlenstoffatomen, eine Arylgruppe mit 6 bis 14 Kohlenstoffatomen oder eine Alkylarylgruppe mit 7 bis 30 Kohlenstoffatomen bedeutet, und
(C) 0,01 bis 10 Gew.-% mindestens eines ungesättigten aliphatischen Alkohols mit 16 bis 24 Kohlenstoffatomen, wobei das Gewichtsverhältnis des ungesättigten aliphatischen Alkohols zu dem Zinkdithiophosphat (C)/(B) 0,1 bis 10 beträgt.

2. Schmierölzusammensetzung gemäß Anspruch 1, die zusätzlich
(D) 0,01 bis 5,0 Gew.-% mindestens eines Detergens-Dispergiermittels enthält.

3. Schmierölzusammensetzung gemäß Anspruch 1 oder 2, worin das Grundschmieröl ein Mineralöl mit einer kinematischen Viskosität von 5 bis 10 000 mm²/s (cSt), gemessen bei 40°C, oder ein synthetisches Öl mit einer kinematischen Viskosität von 5 bis 10 000 mm²/s (cSt), gemessen bei 40°C, ist.

4. Schmierölzusammensetzung gemäß einem der Ansprüche 1 bis 3, in der das Zinkdithiophosphat aus der aus Zink-di-primären (C₃-C₁₂)-alkyldithiophosphaten, Zink-di-sekundären (C₃-C₁₂)-alkyldithiophosphaten und Zink-bis-(C₉-C₂₄)-(alkyl-aryl)-dithiophosphaten bestehenden Gruppe ausgewählt ist.

5. Schmierölzusammensetzung gemäß einem der Ansprüche 1 bis 4, in der der ungesättigte aliphatische Alkohol 11-Docosen -1-ol, 13-Docosen-1-ol, 9-Eicosen-1-ol oder cis-9-Octadecen -1-ol ist.

6. Schmierölzusammensetzung gemäß Anspruch 1 oder 5, in der der ungesättigte aliphatische Alkohol 13-Docosen-1-ol oder cis-9-Octadecen-1-ol ist.

7. Schmierölzusammensetzung gemäß Anspruch 1, in der das Grundschmieröl ein Mineralöl ist, das Zinkdithiophosphat ein Gemisch aus Zink-di-prinmären (C₄-C₈)-alkyldithiophospaten ist und der ungesättigte aliphatische Alkohol cis-9-Octadecen -1-ol ist.

8. Schmierölzusammensetzung gemäß einem der Ansprüche 1 bis 7, die zusätzlich (E) 0,01 bis 5,0 Gew.-% mindestens eines Additivs enthält, das aus der aus Phosphorsäureestern, Phosphorigsäureestern, Aminsalzen von Phosphorsäureestern und Aminsalzen von Phosphorigsäureestern bestehenden Gruppe ausgewählt ist.

9. Schmierölzusammensetzung gemäß Anspruch 2, in der der ungesättigte aliphatische Alkohol 13-Docosen-1-ol ist.

10. Schmierölzusammensetzung gemäß Anspruch 2, in der das Grundschmieröl ein Mineralöl ist, das Zinkdithiophosphat ein Gemisch aus Zink-di-primären-(C₄-C₆)-alkyldithiophosphaten ist, der ungesättigte aliphatische Alkohol 13-Docosen-1-ol ist und das Detergens-Dispergiermittel ein Gemisch aus Calciumsulfonat und Calciumphenat ist.

11. Schmierölzusammensetzung gemäß Anspruch 2, in der das Grundschmieröl ein Mineralöl ist, das Zinkdithiophosphat ein Gemisch aus Zink-di-primären-(C₄-C₆)-alkyldithiophosphaten ist, der ungesättigte aliphatische Alkohol 13-Docosen-1 -ol ist, das Detergens-Dispergiermittel ein Gemisch aus Calciumsulfonat und Calciumphenat ist und das Additiv Tricresylphosphat ist.

## Revendications

1. Composition d'huile lubrifiante, comprenant :
(A) une quantité importante d'au moins une huile lubrifiante de base ;
(B) de 0,05 à 5 % en poids d'au moins un dithiophosphate de zinc ayant une structure représentée par la formule générale (1) suivante dans laquelle chacun des R¹, R², R³ et R⁴ représente indépendamment des autres un groupe alkyle primaire ayant de 2 à 30 atomes de carbone, un groupe alkyle secondaire ayant de 3 à 30 atomes de carbone, un groupe cycloalkyle ayant de 6 à 30 atomes de carbone, un groupe aryle ayant de 6 à 14 atomes de carbone ou un groupe alkylaryle ayant de 7 à 30 atomes de carbone ;
(C) de 0,01 à 10 % en poids d'au moins un alcool aliphatique insaturé ayant de 16 à 24 atomes de carbone ;
le rapport pondéral de l'alcool aliphatique insaturé au dithiophosphate de zinc (C)/(B) étant compris entre 0,1 et 10.

2. Composition d'huile lubrifiante suivant la revendication 1, comprenant en outre :
(D) de 0,01 à 5,0 % en poids d'au moins un détergent-dispersant.

3. Composition d'huile lubrifiante suivant la revendication 1 ou 2, dans laquelle l'huile lubrifiante de base est une huile minérale ayant une viscosité cinématique mesurée à 40°C comprise entre 5 et 10 000 mm²/s (cSt) ou une huile synthétique ayant une viscosité cinématique mesurée à 40°C comprise entre 5 et 10 000 mm²/s (cSt).

4. Composition d'huile lubrifiante suivant l'une quelconque des revendications 1 à 3, dans laquelle le dithiophosphate de zinc est choisi parmi l'ensemble consitué par les di-primaire-(C₃-C₁₂)-alkyldithiophosphates de zinc, di-secondaire-(C₃-C₁₂)-alkyldithiophosphates de zinc et bis-(C₉-C₂₄)-(alkylaryl)dithiophosphates de zinc.

5. Composition d'huile lubrifiante suivant la revendication 1 ou 4, dans laquelle l'alcool aliphatique insaturé est le 11-docosène-1-ol, le 13-docosène-1-ol, le 9-eicosène-1-ol ou le cis-9-octadécène-1-ol.

6. Composition d'huile lubrifiante suivant la revendication 1 ou 5 , dans laquelle l'alcool aliphatique insaturé est le 13-docosène-1-ol ou le cis-9-octadécène-1-ol.

7. Composition d'huile lubrifiante suivant la revendication 1, dans laquelle l'huile lubrifiante de base est une huile minérale, le dithiophosphate de zinc est un mélange de di-primaire-(C₄-C₆)-alkyldithiophosphates de zinc, et l'alcool aliphatique insaturé est le cis-9-octadécène -1-ol.

8. Composition d'huile lubrifiante suivant l'une quelconque des revendications 1 à 7, ladite composition comprenant en outre :
(E) de 0,01 à 5,0 % en poids d'au moins un additif choisi parmi l'ensemble constitué par les esters phosphoriques, esters phosphoreux, sels d'amine d'esters phosphoriques et sels d'amine d'esters phosphoreux.

9. Composition d'huile lubrifiante suivant la revendication 2, dans laquelle l'alcool aliphatique insaturé est le 13-docosène-1-ol.

10. Composition d'huile lubrifiante suivant la revendication 2, dans laquelle l'huile lubrifiante de base est une huile minérale, le dithiophosphate de zinc est un mélange de di-primaire-(C₄ -C₆)-alkyldithiophosphates de zinc, l'alcool aliphatique insaturé est le 13-docosène-1-ol, et le détergent-dispersant est un mélange de sulfonate de calcium et de phénate de calcium.

11. Composition d'huile lubrifiante suivant la revendication 2, dans laquelle l'huile lubrifiante de base est une huile minérale, le dithiophosphate de zinc est un mélange de di-primaire-(C₄-C₆)-alkyldithiophosphates de zinc, l'alcool aliphatique insaturé est le 13-docosène-1-ol, le détergent-dispersant est un mélange de sulfonate de calcium et de phénate de calcium, et l'additif est le phosphate de tricrésyle.
